

(No Model.)

M. L. GRIFFIN & P. O. LARSEN.  
METHOD OF DIGESTING WOOD PULP.

No. 551,890.

Patented Dec. 24, 1895.



WITNESSES—

A. F. Macdonald.

B. D. Hall.

INVENTORS

Martin L. Griffin  
Petter Otto Larsen  
By E. W. Cady  
Atty.

# UNITED STATES PATENT OFFICE.

MARTIN L. GRIFFIN AND PETTER OTTO LARSEN, OF MECHANICSVILLE,  
NEW YORK.

## METHOD OF DIGESTING WOOD PULP.

SPECIFICATION forming part of Letters Patent No. 551,890, dated December 24, 1895.

Application filed November 30, 1894. Serial No. 530,423. (No specimens.)

*To all whom it may concern:*

Be it known that we, MARTIN L. GRIFFIN, a citizen of the United States, and PETTER OTTO LARSEN, a subject of the King of Sweden and

5 Norway, residents of Mechanicsville, county of Saratoga, and State of New York, have invented an Improved Method of Digesting Wood Pulp, of which the following is a specification.

10 This invention relates to digesting wood by the sulphite process.

This invention has for its object economy and simplicity of operation by providing a steady and continuous increase in energy during the operation of cooking, insuring a continuous and steady rise in temperature of the whole mass, and utilizing the excess of gas and liquor during the first part of the operation before the cooking commences, and also 15 utilizing the excess of gas, liquor, and steam during the cooking operation by discharging the same into a succeeding charge of liquor in a tank containing partially-prepared liquor and thereafter supplying the digester with 20 this prepared cooking liquor.

In carrying out this invention it is preferably employed in connection with the well-known process of digesting wood by the sulphite process.

25 In the accompanying drawing is shown an apparatus to illustrate the manner of working this process, consisting of a digester, a tank for containing the partially-prepared cooking liquor, a blow-off pipe connecting the digester with said tank, and so much of the well-known pipe connections as are necessary for setting forth this invention.

A is the digester constructed in the well-known way for digesting wood pulp and provided with the opening B in its top through which the charge of wood is passed into the digester, and having the cover C adapted to be secured over the opening B.

30 In charging the digester it is preferably practically filled with chips of wood and supplied with cooking liquor through any suitable pipe connection—as, for example, the

pipe H shown as broken away and connected with a suitable supply-tank F.

35 I is a blow-off valve for the discharge of 50 the cooked mass.

The cooking liquor is supplied so as to cover the chips of wood, leaving no appreciable space for condensation of steam.

40 The cooking liquor may, for example, be 55 composed of about one and forty one-hundredths to one and fifty one-hundredths per cent. of lime, magnesia or other alkaline base; about one and seventy-five one-hundredths per cent. of combined sulphurous-acid gas, 60 and about two and fifty one-hundredths per cent. to two and seventy-five one-hundredths per cent. of free sulphurous-acid gas.

45 In the commencement of the operation, steam is admitted to the digester through the 65 pipe D from a suitable source. To facilitate the admission of the steam and provide for condensation a pipe E is employed of suitable acid-resisting material, which is connected at one end with the upper end or neck 70 of the digester A and at the other with the storage reservoir or tank F, containing a charge of partially-prepared cooking liquor having about one and fifty one-hundredths 75 percent. of base and one and seventy one-hundredths per cent. of combined and the same amount of free sulphurous-acid gas. This partially-prepared liquor is in this way supercharged with sulphurous-acid gas, which renders the liquor more efficient in the cooking, producing a whiter and more uniformly-cooked mass. The pipe E is provided with a valve G by means of which the flow of liquor, gas, and steam through pipe E from the 80 digester A to the tank F is regulated.

50 As heretofore stated, in the commencement of the operation steam from a battery of boilers is admitted to the digester through pipes D, the valve G is opened and a continuous discharge of liquor and gas from digester A into 85 tank F, containing the partly-prepared cooking liquor, takes place during the first part of the operation, until the temperature of the mass in the digester reaches about 212° Fahr-

enheit, and after said temperature is reached and the cooking commences a continuous discharge of liquor, gas and steam takes place from digester A into the tank F, containing 5 the partially-prepared cooking liquor. During this operation, properly conducted, we are able to raise and maintain the proper pressure and degree of heat by so regulating the valve G that it will discharge only a volume 10 of liquid equivalent to the amount of steam entering the digester through the valve D. For instance, suppose we admit steam to digester at eighty pounds pressure through a three-inch pipe and valve D, the area of whose 15 orifice is seven square inches. It would require an orifice at G whose area was four and nine-tenths square inches to discharge the water of condensation under practically no head, while at the same time the temperature of the 20 contents of the digester would be continuously rising. As soon as a temperature of about 212° Fahrenheit is reached in the digester by closing off the valve G continuously the temperature and pressure will continue 25 to rise until the desired pressure of eighty pounds and its corresponding temperature is reached, when an orifice, as at G, whose area is only twenty-five one-thousandths of a square inch will be ample for the discharge of the 30 condensation of the current of steam entering at full head through the orifice at D, and provided the same would be all condensed, which of course it would not. Neither would it be necessary, but in fact undesirable, to admit 35 a continuous current of steam of a constant quantity during the whole period of cooking.

The amount of liquor to be discharged will be equivalent to the amount of condensation of the steam, which will be about twenty per 40 cent. of the quantity contained in the digester. It will be necessary to relieve the gas and liquor in such quantities continuously as to insure a continuous rise in the temperature of the mass.

45 As the bulk of the condensation takes place in raising the mass to 212° Fahrenheit before the liquor exerts any marked cooking action, the liquor displaced by the condensation of steam is available for a subsequent cooking 50 operation, and the excess of gas discharged simultaneously with the liquor into the tank D will increase the strength of the liquor contained in it from about three and forty one-hundredths per cent. of sulphurous-acid gas 55 to about four and fifty one-hundredths per cent., besides raising the temperature of the same to a considerable degree.

It has been the practice when the pressure in the digester is equal, or nearly so, to the 60 pressure of the steam entering, and the temperature of the contents of the digester does not correspond to the pressure, to relieve an indefinite quantity of the disengaged sulphurous-acid gas, thereby admitting steam afresh and quickly raising the temperature 65 through an indefinite number of degrees, until

the condition of equilibrium of gases and steam-pressure recur, when the blowing off again of gas is resorted to in order to raise the temperature to the proper degree necessary 70 for cooking the wood.

The advantages of our improved process are as follows:

First. At the beginning of the cooking operation we set the steam-valve for the steam 75 entering the digester so as to insure a continuous and steady flow of live steam into the mass to be cooked.

Second. At the same time we open the valve 80 G in the discharge-pipe just enough to discharge a volume of liquor equal to that resulting from the condensation of the entering steam, and thereby insure a continuous and steady rise in temperature of the entire mass.

Third. By our process we carry forward the 85 entire operation of cooking the wood by a steady and continuous increment of energy, including the preparation of and adaptation of the liquor best suited for the mechanical part of the process set forth, thereby eliminating 90 the contingencies and uncertainties attendant upon the present mode of reducing wood to fiber.

Fourth. We are also able to reduce the labor account by the operation of our process, since 95 when steam is turned on properly at the beginning of the cooking and the relief-valve properly adjusted no further labor or attention becomes necessary until near the close of the operation, whereas with the present mode 100 of procedure the constant attention of skilled cooks is required.

Having now described our invention, what we claim is—

1. The herein described method of digesting 105 wood by the sulphite process, which consists in admitting steam to the digester containing a charge of chips and cooking liquor, maintaining a continuous discharge of liquor and gas from the digester into a tank containing 110 partly prepared cooking liquor, until the cooking begins, and then maintaining a continuous admission of steam into the digester and a continuous discharge of liquor, gas and steam from the digester into the tank of partly prepared 115 cooking liquor during the cooking.

2. The method of digesting wood by the sulphite process, which consists in admitting steam to the digester containing a charge of chips and cooking liquor and maintaining 120 from the beginning of, during and to the termination of the cooking, a continuous admission of steam into the digester and a continuous discharge of liquor, gas and steam from the digester into a tank of partly prepared 125 cooking liquor.

3. The herein described method of digesting 130 wood, which consists in filling the digester practically full of chips and cooking liquor covering the chips, admitting steam to the digester, maintaining a continuous discharge of liquor and gas from the digester into a tank

containing partly prepared cooking liquor until the cooking begins, regulating the discharge of steam entering the digester, and maintaining during the cooking a continuous admission of steam into the digester and a continuous discharge of liquor, gas and steam into the tank of partly prepared cooking liquor containing about one and one-half per cent. of lime or other alkaline base, and three and forty one-hundredths per cent. of sulphur-

ous acid gas for the preparation of a fresh charge of cooking liquor.

In witness whereof we have hereunto set our hands this 14th day of November, 1894.

MARTIN L. GRIFFIN.  
PETTER OTTO LARSEN.

Witnesses:

NEWTON T. BRYAN,  
FRANK A. CURLEY.